

July 28, 1970

C. D. McLAIN

3,522,038

COPPER BASE ALLOY

Filed June 26, 1967

2 Sheets-Sheet 1



**FIG - 1**

INVENTOR:  
CHARLES D. McLAIN

BY *Robert N. Bachman*  
ATTORNEY

July 28, 1970

C. D. McLAIN

3,522,038

COPPER BASE ALLOY

Filed June 26, 1967

2 Sheets-Sheet 2



**FIG - 2**

INVENTOR:  
CHARLES D. McLAIN

BY *Robert N. Bachman*  
ATTORNEY

1

3,522,038  
**COPPER BASE ALLOY**  
Charles D. McLain, Alton, Ill., assignor to Olin  
Corporation, a corporation of Virginia  
Filed June 26, 1967, Ser. No. 648,660  
Int. Cl. C22c 9/00, 9/10

U.S. Cl. 75—153

7 Claims

## ABSTRACT OF THE DISCLOSURE

The present disclosure teaches a copper base alloy containing 1.5–3.5% iron, 0.02 to 0.21% silicon, at least one of the elements phosphorous and zinc in amounts 0.01 to 0.15% and 0.03 to 0.2% respectively, as well as other optional additives. The alloys in the present specification are characterized by improved physical properties, in particular high strength and high conductivity.

As is well known in the art, copper is an excellent conductor of electricity. Numerous alloying additions have been proposed in order to increase the strength of copper. In so doing, the electrical conductivity of the copper is markedly reduced.

It is, therefore, highly desirable to provide a copper base alloy characterized by high conductivity and increased strength.

Accordingly, it is a principal object of the present invention to provide a copper base alloy characterized by high electrical conductivity and high strength properties.

It is a further object of the present invention to provide a copper base alloy with annealed physical properties which do not have a wide variation.

It is a further object of the present invention to provide a copper base alloy having the ability to attain various strength levels as a result of different annealing treatments, even when small amounts of impurities are present.

It is a further object of the present invention to provide an improved copper base alloy having a combination of high strength, high conductivity, and other excellent physical properties.

It is an additional object of the present invention to provide a copper base alloy which is inexpensive and wherein the excellent physical properties are easily obtainable.

Further objects and advantages of the present invention will appear from the ensuing specification.

In accordance with the present invention it has been found that an improved copper base alloy is provided which effectively achieves the foregoing objects and advantages. The alloy of the present invention comprises a copper base alloy consisting essentially of from 1.5 to 3.5% iron, 0.02 to 0.21% silicon and the balance essentially copper. In addition, the copper base alloy of the present invention effectively utilizes additional additives such as phosphorus in an amount from 0.01 to 0.15%, preferably from 0.01 to 0.10%, and zinc in an amount from 0.03 to 0.20%, preferably from 0.03 to 0.15%, and mixtures thereof. Throughout the ensuing specification all percentages are percentages by weight.

In accordance with the present invention, it has been surprisingly found that the foregoing alloys are characterized by numerous unexpected and surprising advantages. For example, the alloys of the present invention have an unexpected improvement in electrical conductivity. Namely, there is readily obtained an IACS electrical conductivity in excess of 70% IACS, and a range of 75 to 81% IACS is readily attained. Furthermore, the alloys of the present invention have excellent annealing characteristics, with the ability to attain various strength levels as a result of different annealing treatments. In addition,

2

the alloys of the present invention attain high rolled temper strength levels. Still further the high electrical conductivity of the alloys of the present invention is coupled with excellent annealed tensile strength properties of approximately 65,000 p.s.i. and higher. The strength and physical properties of the alloys of the present invention are not significantly variable if small amounts of impurities are present. Still further the alloys of the present invention resist softening during soldering at 700 to 800° F. In addition to the foregoing, the alloys of the present invention are inexpensive and their excellent physical properties easily obtainable.

The composition of the alloys of the present invention is as stated heretofore. The preferred iron content is from 1.7 to 3.0%, with an optimum from 1.8 to 2.9% and the preferred silicon content is from 0.03 to 0.20% with an optimum range being from 0.10 to 0.17%.

In view of the high and in fact surprising physical properties of the alloys of the present invention, the percentage ranges of the alloying ingredients are important.

In addition to the foregoing, small amounts of additional alloying ingredients may be, of course, included in order to achieve particularly desirable results, for example, aluminum in an amount up to 0.07% and manganese in an amount up to 0.08%. Also, small amounts of impurities may, of course, be tolerated.

The alloys of the present invention attain improvement over conventional alloys in a wide range of processing. Naturally, however, particular processing will result in variation in properties.

The manner of casting the material is not particularly critical, with conventional casting methods for these types of alloys being readily utilizable, it being noted that higher temperatures should be used in order to solutionize the iron. It is preferred to cast the alloy into billets of conventional size, subjecting them to hot working, as by rolling in the conventional size.

After casting the alloy should be hot rolled at an elevated temperature, i.e., from 800 to 1050° C., with a temperature of about 950° C. being preferred. The alloy should then be cold rolled to gage, with intermediate anneals, with cold reduction in excess of 50% between anneals being preferred. Annealing temperatures of from 400 to 600° C. are preferred, with annealing time at temperature preferably being a minimum of two (2) hours. Longer times may be utilized, if desired, for improved electrical conductivity. Continuous strand annealing of strip or mill products will achieve the same high level of physical properties as with Bell annealing, but will not achieve as high a level of electrical conductivity. Therefore, for development of both high annealed strength and electrical conductivity, final annealing and preferably in process annealing must be in batches with conventional furnace cooling, such as Bell annealing.

Detailed processing and preferred processing parameters consonant with the foregoing are found in co-pending application Ser. No. 648,742 for "Process for Treating Copper Base Alloy," filed of even date herewith, by C. D. McLain.

The present invention will be more readily understandable from a consideration of the following illustrative examples.

## EXAMPLE I

Alloys were prepared in the following manner. High purity copper and high purity iron were melted together in a low frequency, slot type induction furnace under a charcoal cover at approximately 1200° C. About 10% of the copper charge was held back and the melt was slightly overheated to about 1300° C. in order to put the iron into solution. High purity alloying additions were

added when the molten mass was at about 1300° C. The balance of the copper was added and the melt brought to the pouring temperature of about 1200° C. The melt was then poured into a water-cooled ingot mold of 28 $\frac{3}{4}$ " x 5" x 96" at a pouring rate of 21.3" per minute.

The alloys thus prepared had the following composition.

and tensile strength. The results are shown in FIGS. 1 and 2. FIG. 1 is a curve of Rockwell 15T hardness versus temperature and FIG. 2 is a curve of strength versus temperature. In FIGS. 1 and 2, the solid lines represent the data after 3 minutes immersion in the salt bath and the dashed lines represent the data after 4

TABLE I

| Alloy  | Iron, percent | Phosphorus, percent | Silicon, percent | Zinc, percent | Copper               |
|--------|---------------|---------------------|------------------|---------------|----------------------|
| 1----- | 2.3           | 0.021               | 0.13             | 0.08          | Essentially balance. |
| 2----- | 2.3           | 0.03                | -----            | -----         | Do.                  |

## EXAMPLE II

Alloys 1 and 2 prepared in Example I were processed as follows. The alloys were hot rolled at from 900 to 940° C., followed by a water spray quench to room temperature. The materials were then cold rolled to 0.100", bell annealed at 480-600° C. (1 to 4 hours at temperature), cold rolled to 0.050", bell annealed at 460 to 480° C. (1 to 3 hours at temperature), and cold rolled to 0.025" gage and bell annealed at 440 to 480° C. (1 to 3 hours at temperature).

15 minutes immersion in the salt bath. There was no change in electrical conductivity of any of the alloys.

These graphs vividly demonstrate that alloy 3, the alloy of the present invention, is markedly and surprisingly superior to conventional alloys 4 and 5.

## EXAMPLE IV

20 In this example three alloys were prepared in a manner after Example I, wherein the alloys had the following compositions:

TABLE IV

| Alloy  | Phosphorus, percent | Iron, percent | Silicon, percent | Zinc, percent | Copper               |
|--------|---------------------|---------------|------------------|---------------|----------------------|
| 6----- | 0.021               | 2.3           | 0.13             | 0.08          | Essentially balance. |
| 7----- | -----               | 2.4           | 0.14             | -----         | Do.                  |
| 8----- | 0.025               | 2.4           | -----            | -----         | Do.                  |

The alloys were then tested for physical properties, with the results being shown in the following table.

TABLE II

| Alloy  | Yield Strength, p.s.i. | Tensile Strength, p.s.i. | Elongation, percent | Electrical Conductivity, percent IACS |
|--------|------------------------|--------------------------|---------------------|---------------------------------------|
| 1----- | 26,900                 | 53,400                   | 27                  | 81.2                                  |
| 2----- | 23,100                 | 50,100                   | 27.5                | 73.5                                  |

35 The alloys were processed in the following manner. The five inch thick slabs were hot rolled at 925° C. to 0.350", milled to 0.300", cold rolled to 0.100", annealed for two hours at 490° C., cold rolled to 0.050", annealed at 440° C. for two hours and cold rolled to 0.025" and annealed for two hours at 440° C.

40 After each anneal the tensile strength and electrical conductivity of each sample was determined and the results are shown in the following table.

TABLE V

| Alloy  | First Anneal             |                                       | Second Anneal            |                                       | Third Anneal             |                                       |
|--------|--------------------------|---------------------------------------|--------------------------|---------------------------------------|--------------------------|---------------------------------------|
|        | Tensile Strength, p.s.i. | Electrical Conductivity, percent IACS | Tensile Strength, p.s.i. | Electrical Conductivity, percent IACS | Tensile Strength, p.s.i. | Electrical Conductivity, percent IACS |
| 6----- | 61,600                   | 69.7                                  | 66,200                   | 73.5                                  | 67,300                   | 76.9                                  |
| 7----- | 56,000                   | 66.2                                  | 63,000                   | 75.1                                  | 66,800                   | 82.0                                  |
| 8----- | 45,100                   | 69.9                                  | 56,000                   | 72.1                                  | 51,100                   | 72.3                                  |

55 the foregoing demonstrates that alloy 1, the alloy of the present invention, achieves higher electrical conductivity than conventional alloy 2, and also develops greater annealed strength levels.

## EXAMPLE III

In this example three alloys were prepared in a manner after Example I, wherein the alloys had the following compositions:

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

TABLE III

| Alloy  | Iron, percent | Silicon, percent | Phosphorus, percent | Silver, percent | Oxygen, percent | Copper               |
|--------|---------------|------------------|---------------------|-----------------|-----------------|----------------------|
| 3----- | 2.4           | 0.12             | -----               | -----           | -----           | Essentially balance. |
| 4----- | 2.4           | -----            | 0.02                | -----           | Do.             | Do.                  |
| 5----- | -----         | -----            | -----               | 0.06            | 0.04            | Do.                  |

The alloys were then processed in a manner after Example II, with an additional cold rolling to increase strength level, and then tested for softening temperature in the following manner. The alloys were immersed in a salt bath at elevated temperatures from 600 to 800° F. for periods of time of 3 and 4 minutes. The samples were then tested for Rockwell 15T hardness, yield strength

70 What is claimed is:

1. A copper base alloy consisting essentially of from 1.5 to 3.5% iron, from 0.02 to 0.21% silicon, at least one of the elements P and Zn, P being present in an amount of 0.01 to 0.15% and Zn being present in an amount of 0.03 to 0.2% Zn, balance copper, said alloy having an IACS electrical conductivity of over 70%,

said alloy being in the rolled temper and having an annealed tensile strength of at least 65,000 p.s.i.

2. A copper base alloy consisting essentially of from 1.5 to 3.5% iron, from 0.02 to 0.21% silicon, from 0.01 to 0.15% phosphorus and the balance copper.

3. A copper base alloy consisting essentially of from 1.5 to 3.5% iron, from 0.02 to 0.21% silicon, from 0.03 to 0.20% zinc and the balance copper.

4. A copper base alloy according to claim 3 containing from 0.01 to 0.15% phosphorus.

5. A copper base alloy according to claim 4 having an IACS electrical conductivity of over 70%, being in the cold rolled and annealed temper and having an annealed tensile strength at least 65,000 p.s.i.

6. A copper base alloy according to claim 4 wherein the silicon is present in an amount from 0.03 to 0.20%, the iron is present in an amount from 1.7 to 3.0%, the phosphorus is present in an amount from 0.01 to 0.10% and the zinc is present in an amount from 0.03 to 0.15%.

7. A copper base alloy according to claim 4 wherein

the silicon is present in an amount from 0.10 to 0.17% and the iron is present in an amount from 1.8 to 2.9%.

## References Cited

## UNITED STATES PATENTS

|           |         |                |          |
|-----------|---------|----------------|----------|
| 1,778,668 | 10/1930 | Fuller         | 75—160   |
| 2,155,406 | 4/1939  | Crampton et al | 75—157.5 |
| 3,039,867 | 6/1962  | McLain         | 75—153   |

## FOREIGN PATENTS

|         |        |                |
|---------|--------|----------------|
| 256,457 | 8/1926 | Great Britain. |
|---------|--------|----------------|

## OTHER REFERENCES

Transactions of AIME, vol. 188, December 1950, pp. 1486, 1487, 1495 and 1498.

CHARLES N. LOVELL, Primary Examiner

U.S. CL. X.R.

20 75—157.5, 160; 148—32.5